



US008877646B2

(12) **United States Patent**  
Marty et al.

(10) **Patent No.:** US 8,877,646 B2  
(45) **Date of Patent:** Nov. 4, 2014

(54) **FILM STACKS AND METHODS THEREOF**

(75) Inventors: **Valerie J Marty**, Corvallis, OR (US);  
**Galen P. Cook**, Albany, OR (US)

(73) Assignee: **Hewlett-Packard Development Company, L.P.**, Houston, TX (US)

(\*) Notice: Subject to any disclaimer, the term of this patent is extended or adjusted under 35 U.S.C. 154(b) by 0 days.

(21) Appl. No.: **13/640,694**

(22) PCT Filed: **Apr. 19, 2010**

(86) PCT No.: **PCT/US2010/031565**

§ 371 (c)(1),  
(2), (4) Date: **Oct. 11, 2012**

(87) PCT Pub. No.: **WO2011/133133**

PCT Pub. Date: **Oct. 27, 2011**

(65) **Prior Publication Data**

US 2013/0034703 A1 Feb. 7, 2013

(51) **Int. Cl.**  
**H01L 21/302** (2006.01)  
**B41J 2/16** (2006.01)

(52) **U.S. Cl.**  
CPC ..... **B41J 2/1601** (2013.01); **B41J 2/1628** (2013.01)

USPC ..... 438/696; 438/724; 438/740; 216/27;  
216/67; 216/72

(58) **Field of Classification Search**

None  
See application file for complete search history.

(56) **References Cited**

U.S. PATENT DOCUMENTS

2005/0174390 A1 8/2005 Sun et al.  
2007/0042113 A1 2/2007 Ji et al.  
2009/0027450 A1 1/2009 Park et al.  
2009/0294810 A1\* 12/2009 Stadel et al. ..... 257/288

OTHER PUBLICATIONS

International Search Report and Written Opinion, Application No. PCT/US2010/031565, Dated Dec. 29, 2010, pp. 9.

\* cited by examiner

*Primary Examiner* — Anita Alanko

(57) **ABSTRACT**

A method of manufacturing a plurality of spacers in a film stack includes forming at least one electrically-conductive element having sidewalls on a substrate, depositing a plurality of passivation layers proximate to the substrate, and performing etching on one of the plurality of passivation layers to form a plurality of spacers substantially across from the sidewalls of the at least one electrically-conductive element.

15 Claims, 5 Drawing Sheets





*FIG. 1A*



*FIG. 1B*



FIG. 1C



FIG. 1D



FIG. 2





FIG. 4A



FIG. 4B



FIG. 4C



FIG. 4D



FIG. 4E



FIG. 4F

## FILM STACKS AND METHODS THEREOF

## BACKGROUND OF THE DISCLOSURE

Film stacks including several layers are used with a thermal fluid ejector apparatus. Such film stacks, for example, are used in thermal inkjet print heads in order to eject ink droplets through the collapse of bubbles formed by heating the ink.

## DESCRIPTION OF THE DRAWINGS

Exemplary non-limiting embodiments of the general inventive concept are described in the following description, read with reference to the figures attached hereto and do not limit the scope of the claims. In the figures, identical and similar structures, elements or parts thereof that appear in more than one figure are generally labeled with the same or similar references in the figures in which they appear. Dimensions of components and features illustrated in the figures are chosen primarily for convenience and clarity of presentation and are not necessarily to scale. Referring to the attached figures:

FIG. 1A is a side view illustrating a film stack usable with a thermal fluid ejector apparatus according to an example embodiment of the present general inventive concept.

FIG. 1B is a side view illustrating a film stack usable with a thermal fluid ejector apparatus according to another example embodiment of the present general inventive concept.

FIG. 1C is a side view of the film stack of FIG. 1A including an etch stop layer according to an example embodiment of the present general inventive concept.

FIG. 1D is a side view of the film stack of FIG. 1B including an etch stop layer according to an example embodiment of the present general inventive concept.

FIG. 2 is a flowchart illustrating a method of manufacturing a plurality of spacers in a film stack according to an example embodiment of the present general inventive concept.

FIGS. 3A-3F are sequential views illustrating the method of manufacturing a plurality of spacers as illustrated in FIG. 2 according to an example embodiment of the present general inventive concept.

FIGS. 4A-4F are sequential views illustrating the method of manufacturing a plurality of spacers as illustrated in FIG. 2 according to an example embodiment of the present general inventive concept.

## DETAILED DESCRIPTION

The present general inventive concept is directed toward a film stack usable with a thermal fluid ejector apparatus and a method of manufacturing a plurality of spacers in the film stack. The thermal fluid ejector apparatus may be, for example, a thermal inkjet print head to eject ink droplets through the collapse of bubbles formed by heating the ink. The film stack, for example, may include a substrate, resistors and conductive interconnect lines each having sidewalls, several passivation layers, and a plurality of spacers formed from one of the passivation layers. The spacers are disposed substantially across from the respective sidewalls of the resistors and conductive interconnect lines.

In accordance with the present general inventive concept, the plurality of spacers are formed from a passivation layer through etching and disposed substantially across from the respective sidewalls of the resistors and conductive interconnect lines. Such an arrangement of spacers, for example, increase dielectric thickness to the sidewalls of the respective

electrically-conductive element and improve step coverage. The spacers of the present general inventive concept enable thin passivation layers to cover the respective topography as compared to conventional film stacks which include a thicker passivation layer susceptible to thin spots due to poor coverage over rough topography. The more conformal passivation layers also prevent seams from forming a direct chemical path to the resistors and conductive interconnect lines resulting in chemical protection and electrical isolation.

FIG. 1A is a side view illustrating a film stack usable with a thermal fluid ejector apparatus according to an example embodiment of the present general inventive concept. FIG. 1B is a side view illustrating a film stack usable with a thermal fluid ejector apparatus according to another example embodiment of the present general inventive concept. Referring to FIGS. 1A and 1B, in the present examples, a film stack 10a and 10b includes a substrate 11, at least one electrically-conductive element 12 having sidewalls 12a disposed on the substrate 11, and a plurality of passivation layers including an electrical insulator passivation layer 14b configured to provide electrical insulation and a chemical insulator passivation layer 14c configured to provide chemical insulation. In the present example, the electrical insulator passivation layer 14b includes a dielectric film of Silicon Nitride (SiN) which has good deposition coverage over topography and the chemical insulator passivation layer 14c includes a dielectric film of Silicon Carbide (SiC) which is resistant to chemical attack.

Referring to FIGS. 1A and 1B, in an example, the at least one electrically-conductive element 12 includes at least one of a resistor and an electrically-conductive interconnect line having sidewalls 12a and the plurality of spacers 14a' formed from one of the plurality of passivation layers and disposed substantially across from the sidewalls 12a of the at least one electrically-conductive element 12. For example, a passivation layer 14a (FIGS. 3C and 4D) is etched to form spacers 14a'. In an example, a thickness of the spacers 14a' is set by a thickness of the passivation layer 14a. Such spacers 14a', for example, increase dielectric thickness to the sidewalls 12a of the respective electrically-conductive element 12 and improve step coverage. In the present example, the plurality of spacers 14a includes rounded top portions.

Such spacers 14a' enable thin passivation layers, for example, by decoupling a thickness of the electrical insulator passivation layer 14b to the sidewalls 12a of the respective electrically-conductive element 12 from the electrical insulator passivation layer 14b above the respective electrically-conductive element 12. The spacers 14a' also prevent seams from forming a direct chemical path to the at least one electrically-conductive element 12 resulting in robust electrical isolation and protection from chemical attack. Thus, in the present example, the spacers 14a' allow for the electrical insulator passivation layer 14b to be thin and provide improved thermal performance, while offering improved chemical and mechanical robustness of the electrically-conductive element 12.

In an example, as illustrated in FIG. 1A, the spacers 14a' of the film stack 10a are disposed in contact with the substrate 11, the at least one of a resistor and an electrically-conductive interconnect line, and the electrical insulator passivation layer 14b. Also, the electrical insulator passivation layer 14b of the film stack 10a is in contact with the substrate 11, the plurality of spacers 14a, the at least one electrically-conductive element 12 and the chemical insulator passivation layer 14c. In the present example, the spacers 14a' are formed from a passivation layer 14a, for example, including SiN. In an

example, the chemical insulator passivation layer **14c** include SiC, and the spacers **14a'** and the electrical insulator passivation layer **14b** include SiN.

FIG. 1C is a side view of the film stack of FIG. 1A including an etch stop layer according to an example embodiment of the present general inventive concept. The film stack **10c** illustrated in FIG. 1C includes the film stack **10a** illustrated in FIG. 1A with the addition of an etch stop layer **13** configured to provide chemical insulation and function as a stop layer in formation of spacers **14a'** through etching. Referring to FIG. 1C, in the present example, the etch stop layer **13** of the film stack **10c** is disposed in contact with the substrate **11**, the at least one of a resistor and an electrically-conductive interconnect line, the plurality of spacers **14a'** and the electrical insulator passivation layer **14b**. Also, in the present example, the electrical insulator passivation layer **14b** of the film stack **10a** is in contact with the etch stop layer **13**, the plurality of spacers **14a'**, and the chemical insulator passivation layer **14c**. In the present example, the spacers **14a'** are formed from a passivation layer **14a**, for example, including SiN. In an example, the etch stop layer **13** and the chemical insulator passivation layer **14c** include SiC, and the spacers **14a'** and the electrical insulator passivation layer **14b** include SiN.

In an example as illustrated in FIG. 18, the electrical insulation passivation layer **14b** of the film stack **10b** is disposed in contact with the substrate **11**, at least one electrically-conductive element **11** the electrical insulator passivation layer **14b**, the plurality of spacers **14a'**, and the chemical insulator passivation layer **14c**.

FIG. 1D is a side view of the film stack usable of FIG. 1B including an etch stop layer according to an example embodiment of the present general inventive concept. The film stack **10d** illustrated in FIG. 10 includes the film stack **10b** illustrated in FIG. 1B with the addition of an etch stop layer **13** configured to provide chemical insulation and function as a stop layer in formation of spacers **14a'** through etching. Referring to FIG. 1D, in the present example, the etch stop layer **13** of the film stack **10d** is disposed in contact with plurality of spacers **14a'**, the electrical insulator passivation layer **14b** and the chemical insulator passivation layer **14c**. Also, in the present example, the electrical insulator passivation layer **14b** is in contact with the substrate **11**, the electrically-conductive element **12** and the etch stop layer **13**, and the chemical insulator passivation layer **14c** is in contact with the plurality of spacers **14a'** and the etch stop layer **13**. In the present example, the spacers **14a'** are formed from a passivation layer **14a**, for example, including SiN. In an example, the etch stop layer **13** and the chemical insulator passivation layer **14c** include SiC, and the spacers **14a'** and the electrical insulator passivation layer **14b** include SiN.

FIG. 2 is a flowchart illustrating a method of manufacturing a plurality of spacers in a film stack according to an example embodiment of the present general inventive concept. Referring to FIG. 2, in block **S210**, at least one electrically-conductive element having sidewalls on a substrate is formed. In an example, the at least one electrically-conductive element may include at least one of a resistor and an electrically-conductive interconnect line. In block **S220**, a plurality of passivation layers is deposited proximate to the substrate. In block **S230**, etching on one of the plurality of passivation layers is performed to form a plurality of spacers substantially across from the sidewalls of the at least one electrically-conductive element. In an example, the method of manufacturing a plurality of spacers may further include an etch stop layer being deposited proximate to the substrate.

FIGS. 3A-3F are sequential views illustrating the method of manufacturing a plurality of spacers as illustrated in FIG. 2

according to an example embodiment of the present general inventive concept. Referring to FIG. 3A, at least one electrically-conductive element **12** having sidewalls **12a** on a substrate **11** is formed. In an example, the at least one electrically-conductive element **12** may include at least one of a resistor, for example having a thickness of approximately 4000 angstroms and an electrically-conductive interconnect line, for example, having a thickness of 6000 angstroms formed by photo and etch processes.

As illustrated in FIG. 3B, an etch stop layer **13** may be deposited proximate to the substrate **11**. In this example, depositing an etch stop layer **13** proximate to the substrate **11** may include depositing the etch stop layer **13** in contact with the substrate **11** and the at least one electrically-conductive element **12** as illustrated in FIG. 3B. The etch stop layer **13** is configured to function as a stop layer, for example, for etching such as anisotropically dry etching to form the spacers **14a'** and provide chemical isolation. In an example, the etch stop layer **13** may include SiC and have a thickness of approximately 100 angstroms. One of the plurality of passivation layers, that is, the spacer passivation layer **14a**, in contact with the etch stop layer **13** may be in the form of a plurality of spacers **14a'** as illustrated in FIG. 3E.

Referring to FIGS. 3C-3F, depositing a plurality of passivation layers proximate to the substrate **11** may include depositing a spacer passivation layer **14a**, for example, on the etch stop layer **13** to be formed into the plurality of spacers **14a'** (FIG. 3C), depositing an electrical isolator passivation layer **14b** on the plurality of spacers **14a'** (FIG. 3E), and depositing a chemical isolator passivation layer **14c** on the electrical isolator passivation layer **14b** (FIG. 3F). Thus, for example, the film stack **100** illustrated in FIG. 10 is formed. In an example, the spacer passivation layer **14a** may have a thickness of 1675 angstroms prior to it being form into the spacers **14a'**. In an example, the electrical isolator passivation layer **14b** may have a thickness of approximately 1675 angstroms. Referring to FIGS. 3C and 3D, in an example, performing etching on one of the plurality of passivation layers **14a** to form a plurality of spacers **14a'** substantially across from the sidewalls **12a** may include anisotropically dry etching the spacer passivation layer **14a** to form the plurality of spacers **14a'**, for example, having rounded top portions substantially across from the sidewalls **12a**. In the present example, the spacer passivation layer **14a** and the electrical isolator passivation layer **14b** may include a same material, for example, SiN. In an example, the chemical isolator passivation layer **14c** may include SiC and have a thickness, for example, 725 angstroms, to increase the passivation layers to a thickness to maintain performance of the at least one electrically-conductive element **12**.

FIGS. 4A-4F are sequential views illustrating the method of manufacturing a plurality of spacers **14a'** as illustrated in FIG. 2 according to an example embodiment of the present general inventive concept. Referring to FIG. 4A, at least one electrically-conductive element **12** having sidewalls **12a** on a substrate **11** is formed. In an example, the at least one electrically-conductive element **12** may include at least one of a resistor, for example having a thickness of approximately 4000 angstroms and an electrically-conductive interconnect line, for example, having a thickness of 6000 angstroms formed by photo and etch processes. As illustrated in FIG. 4B, in an example, depositing the plurality of passivation layers proximate to the substrate **11** may include depositing an electrical isolator passivation layer **14b** on the substrate **11** and the at least one of the resistor and the electrically-conductive interconnect line. In an example, the electrical isolator passivation layer **14b** may include SiN and have a thickness of

approximately 1675 Å. Referring to FIG. 40, depositing an etch stop layer 13 proximate to the substrate 11 may include depositing the etch stop layer 13 between and in contact with the spacer passivation layer 14a and the electrical isolator passivation layer 14b. The etch stop layer 13 is configured to function as a stop layer, for example, for etching such as anisotropically dry etching to form the spacers 14a' and provide chemical isolation. In an example, the etch stop layer 13 may include SiC and have a thickness of approximately 100 angstroms.

Referring to FIG. 4D, depositing the plurality of passivation layers proximate to the substrate 11 may also include depositing a spacer passivation layer 14a, for example, on the etch stop layer 13 such that the spacer passivation layer 14a is to be formed into a plurality of spacers 14a' as illustrated in FIG. 4E. In an example, top portion of the spacers 14a' has a rounded top portion. In an example, the spacer passivation layer 14a may have a thickness of 1675 angstroms prior to it being formed into the spacers 14a'. Performing etching on one passivation layer, that is the spacer passivation layer 14a, to form a plurality of spacers 14a' substantially across from the sidewalls 12a may include anisotropically dry etching the spacer passivation layer 14a to form the plurality of spacers 14a', for example, having rounded top portions substantially across from the sidewalls 12a.

Referring to FIG. 4F, depositing the plurality of passivation layers proximate to the substrate 11 may also include and depositing a chemical isolator passivation layer 14c on the spacer passivation layer 14a which is in the form of the plurality of spacers 14a'. Thus, for example, the film stack 10d illustrated in FIG. 1D is formed. In the present example, the spacer passivation layer 14a and the electrical isolator passivation layer 14b may include a same material, for example, SiN. In an example, the chemical isolator passivation layer 14c may include SiC and have a thickness, for example, 725 angstroms, to bring the passivation layers up to a thickness to maintain performance of the at least one electrically-conductive element 12.

The present general inventive concept has been described using non-limiting detailed descriptions of embodiments thereof that are provided by way of example and are not intended to limit the scope of the general inventive concept. It should be understood that features and/or operations described with respect to one embodiment may be used with other embodiments and that not all embodiments of the general inventive concept have all of the features and/or operations illustrated in a particular figure or described with respect to one of the embodiments. Variations of embodiments described will occur to persons of the art. Furthermore, the terms "comprise," "include," "have" and their conjugates, shall mean, when used in the disclosure and/or claims, "including but not necessarily limited to."

It is noted that some of the above described embodiments may describe examples contemplated by the inventors and therefore may include structure, acts or details of structures and acts that may not be essential to the general inventive concept and which are described as examples. Structure and acts described herein are replaceable by equivalents, which perform the same function, even if the structure or acts are different, as known in the art. Therefore, the scope of the general inventive concept is limited only by the elements and limitations as used in the claims.

What is claimed is:

1. A method of manufacturing a plurality of spacers in a film stack, comprising:

forming at least one electrically-conductive element having sidewalls on a substrate;

depositing an etch stop layer at one side of the substrate; depositing a plurality of passivation layers at the one side of the substrate, the plurality of passivation layers including a spacer passivation layer and an electrical isolator passivation layer; and

performing etching of the spacer passivation layer to form a plurality of spacers substantially across from the sidewalls of the at least one electrically-conductive element, the etch stop layer interposed between the at least one electrically-conductive element and the plurality of spacers, and in contact with the plurality of spacers and the electrical isolator passivation layer,

the etch stop layer and the electrical isolator passivation layer coextensively extended along the one side of the substrate.

2. The method according to claim 1, wherein the at least one electrically-conductive element comprises:  
at least one of a resistor and an electrically-conductive interconnect line.

3. The method according to claim 1, wherein the etch stop layer is in contact with the electrical isolator passivation layer along a length of the one side of the substrate.

4. The method according to claim 1, wherein depositing an etch stop layer at one side of the substrate comprises:  
depositing the etch stop layer in contact with the substrate and the at least one electrically-conductive element.

5. The method according to claim 4, wherein depositing a plurality of passivation layers at the one side of the substrate comprises:  
depositing the spacer passivation layer on the etch stop

layer; and  
after performing etching of the spacer passivation layer to form the plurality of spacers, depositing the electrical isolator passivation layer on the etch stop layer and the plurality of spacers.

6. The method according to claim 5, wherein depositing a plurality of passivation layers at the one side of the substrate further comprises:

depositing a chemical isolator passivation layer on the electrical isolator passivation layer.

7. The method according to claim 1, wherein depositing an etch stop layer at one side of the substrate comprises:  
depositing the etch stop layer on the electrical isolator passivation layer.

8. The method according to claim 7, wherein depositing a plurality of passivation layers at the one side of the substrate comprises:  
depositing the electrical isolator passivation layer in contact with the substrate and the at least one electrically-conductive element.

9. The method according to claim 8, wherein depositing a plurality of passivation layers at the one side of the substrate further comprises:  
after performing etching of the spacer passivation layer to form the plurality of spacers, depositing a chemical isolator passivation layer on the etch stop layer and the plurality of spacers.

10. The method according to claim 1, wherein performing etching of the spacer passivation layer to form a plurality of spacers comprises:  
anisotropically dry etching the spacer passivation layer to form the plurality of spacers having rounded top portions substantially across from the sidewalls.

11. The method according to claim 1, the at least one electrically-conductive element having the sidewalls and an end wall, the etch stop layer and the electrical isolator passi-

vation layer coextensively extended along the sidewalls and the end wall of the at least one electrically-conductive element.

**12.** A method of manufacturing a plurality of spacers in a film stack, comprising:

forming at least one electrically-conductive element having opposite sidewalls on a substrate;  
 forming an etch stop layer at one side of the substrate;  
 forming a plurality of spacers at the opposite sidewalls of the at least one electrically-conductive element; and  
 forming an electrical isolator passivation layer at the one side of the substrate,  
 the etch stop layer interposed between the at least one electrically-conductive element and the plurality of spacers, and in contact with the plurality of spacers and the electrical isolator passivation layer,  
 the etch stop layer and the electrical isolator passivation layer commensurately extended at the one side of the substrate.

**13.** The method according to claim **12**, wherein forming an etch stop layer at one side of the substrate comprises depos-

iting the etch stop layer in contact with the substrate and the at least one electrically-conductive element, and wherein forming an electrical isolator passivation layer at the one side of the substrate comprises depositing the electrical isolator passivation layer on the etch stop layer and the plurality of spacers.

**14.** The method according to claim **12**, wherein forming an etch stop layer at one side of the substrate comprises depositing the etch stop layer on the electrical isolator passivation layer, and wherein forming an electrical isolator passivation layer at the one side of the substrate comprises depositing the electrical isolator passivation layer in contact with the substrate and the at least one electrically-conductive element.

**15.** The method according to claim **12**, the at least one electrically-conductive element having the opposite sidewalls and an end wall, the etch stop layer and the electrical isolator passivation layer commensurately extended at the opposite sidewalls and the end wall of the at least one electrically-conductive element.

\* \* \* \* \*